

Patented Aug. 3, 1926.

## UNITED STATES PATENT OFFICE.

ALADAR PACZ, OF CLEVELAND, OHIO, ASSIGNEE TO ALUMINUM COMPANY OF AMERICA, OF PITTSBURGH, PENNSYLVANIA, A CORPORATION OF PENNSYLVANIA.

## ALLOY.

No Drawing.

Application filed December 19, 1924. Serial No. 757,040.

My invention relates to aluminum base alloys containing silicon and other metals and possessing the capability of having their grain refined and physical properties improved by an alkali metal treatment. More especially it relates to an aluminum base alloy containing copper, manganese and a substantial amount of silicon.

In my prior Letters Patent No. 1,387,900, I disclosed an aluminum base alloy containing silicon which had had its grain refined and its physical properties improved by an alkali metal treatment involving treating the molten metal with a fluorine compound of an alkali metal. Another alkali metal treatment for similarly improving aluminum silicon alloys has been disclosed in Patent No. 1,410,461. Aluminum silicon alloys which have been subjected to an alkali metal treatment are generally referred to as "modified" alloys.

My present invention is based on the discovery that aluminum silicon alloys containing small amounts of copper and manganese are not only susceptible to improvement by an alkali metal treatment with the attendant retention of the fluidity and much of the ductility of such alloys but when so treated possess greatly increased tensile strength and hardness as compared with aluminum silicon alloys.

As a specific illustration of my invention, an alloy containing about 12% of silicon, 1/2% of manganese and 1 1/4% copper, the balance being commercial aluminum, was subjected to an alkali metal treatment and cast in a permanent mold. It attained a tensile strength of about 41,000 pounds per square inch and an elongation of about 4 1/2% in two inches, both as measured in standard test bars. These maximum properties were retained during several remelting and recasting operations without further subjecting of the molten metal to the alkali treatment.

Another alloy containing about 12% silicon, 1% copper and 1/4% manganese, with the balance commercial aluminum, when subjected to the alkali metal treatment and cast in a permanent mold, attained a tensile strength of about 41,000 pounds per square inch and an elongation of about 6 1/4% in two inches. This alloy also retained the at-

tained strength and elongation during remelting and recasting operations without being further subjected to the alkali metal treatment but, as was the case with the above composition, gradually lost the same as the reaction products of that treatment were eliminated from the alloy.

I have found that copper and manganese in certain amounts may be employed advantageously with aluminum base alloys containing between about 3% and about 15% of silicon. The copper may vary between about 1/2% and 3% and the manganese may vary between about 1/10% and 1%. The properties desired in any casting of this alloy will, of course, determine to some extent the amount and proportion of the copper, silicon and manganese to be employed but where good tensile strength and fluidity and fair elongation are desired, I prefer to use about 12% of silicon, 1 1/2% of copper and about 1/2% of manganese. Such an alloy will, when cast in a permanent mold, possess a hardness of about 70 Brinell, which is higher than the hardness of most improved or modified silicon alloys known heretofore.

Various additional metals such as cobalt, uranium, tungsten, molybdenum may be added in small quantities to the foregoing alloys without harmful effect on the properties of the alloys as described hereinabove.

Having thus described my invention, what I desire to secure by Letters Patent is defined in what is claimed.

What I claim is:

1. An aluminum base alloy containing between about 3% and about 15% of silicon, and copper and manganese totalling from about 0.75% to 4% the copper constituting at least about 0.5% of the alloy.

2. An aluminum base alloy containing between about 3% and about 15% of silicon, between about 0.5% and 3% of copper and between about 0.25% and about 1.0% of manganese.

3. An aluminum base alloy containing between about 3% and about 15% of silicon, between about 1.0% and 1.5% of copper and about 0.5% of manganese.

4. An aluminum base alloy containing 3% to 15% of silicon, 1.0% to 1.5% of copper and 0.5% of manganese.

- 2
5. An aluminum base alloy containing 12% silicon, 1.25% of copper and 0.5% manganese.
  6. A modified aluminum base alloy containing copper in appreciable amounts not exceeding about 3%, manganese in appreciable amounts not exceeding about 1%, and between about 8% and about 15% of silicon

and characterized, when cast in a permanent mold, by having a tensile strength of about 10,40,000 lbs. per square inch, an elongation of about 4%, and a hardness of about 70 Brinell.

In testimony whereof I hereunto affix my signature this 16th day of December, 1924.

ALADAR PACZ.